

# UNITED STATES PATENT OFFICE.

CHARLES LE PETIT, OF MOMBASA, BRITISH EAST AFRICA, ASSIGNOR TO POWER  
ALCOHOL LIMITED, OF LONDON, ENGLAND.

## FUEL.

1,377,992.

Specification of Letters Patent. Patented May 10, 1921.

No Drawing.

Application filed September 18, 1919. Serial No. 324,296.

To all whom it may concern:

Be it known that I, CHARLES LE PETIT, a citizen of the French Republic, residing at Mombasa, British East Africa, have invented certain new and useful Improvements in Fuels, of which the following is a specification.

This invention relates to fuels and to the production thereof, and has for its object to 10 provide an improved combustible particularly adaptable for use in internal-combustion engines.

With some fuels which, upon combustion, give rise to acidic bodies, it has been proposed to use certain basic additions for the purpose of neutralizing these acidic bodies. Thus ammonia has been so employed, one known fuel consisting of alcohol, ether and this base, together with a trace of white 20 arsenic, presumably for denaturation. The ammonia has been introduced in the gaseous form, and alternatively in concentrated aqueous solutions, but in both cases is objectionable by reason of its action on metallic 25 parts, such as those of copper, nickel and aluminium. To avoid the disadvantages associated with ammonia, trimethylamin has been substituted, and it has similarly been proposed to improve the qualities of liquid 30 fuels by passing into them ammonia derivatives of hydrocarbons, such as methylamin, under pressure. The amins are for the most part very readily soluble in alcohol, and the use of pressure results in a strong solution, 35 and the presence in the fuel in substantial proportions of these powerful bases is not only detrimental, but quite unnecessary. The odor of the fuel is objectionable, and that from the exhaust of the engine particularly so, a disadvantage which is also 40 associated with the use of ammonia. It is the purpose of this invention to provide a fuel in which the production of acidic bodies is inhibited, and the neutralization of such 45 as are formed readily effected, while at the same time the objectionable odor from the engine's exhaust is obviated, these advantages being attained without reduction in the explosive power of the fuel.

50 According to the present invention, in the production of a liquid fuel, such as a fuel

for internal-combustion engines, there is employed a comparatively small proportion of one or more aliphatic amines, together with one or more esters of formic acid, such 55 as ethyl- or methyl-formate. Preferably methylamines, for example mono- and di-methylamin, are employed. The invention is particularly adaptable to fuels which consist of or contain alcohol and ether, and 60 according to one embodiment of the invention the improved fuel comprises ethyl alcohol, ether, an aliphatic amine, or mixture of amines, and a formyl-ester, such as ethyl- 65 or methyl-formate.

Where more than one amine is employed, these need not belong to the same aliphatic series, for example, a mixture of methylamines and ethylamines may be utilized. A natural source of such a mixture is vinasse, 70 a by-product in the manufacture of beet sugar. Similarly a mixture of methylamines may be obtained from herring brine. The addition of the bases may be made in any 75 suitable way. Thus, gaseous methylamin may be dissolved in the other ingredients of the fuel, such as the mixture of alcohol and ether, or mono-methylamin in the liquid form may be added.

The proportions of amines used depend 80 upon circumstances, such as the nature of the other constituents of the fuel and its particular composition. For many purposes these proportions will be found to be in the neighborhood of 0.5 to 2%. The 85 esters may be used in approximately the same proportions as the amines, or sometimes in rather larger amounts. Generally it will be found that a smaller proportion of ester than of amine should be used, advantageously half as much of a 50% mixture of methyl- and ethyl-formate.

As illustrative of the invention the following examples may be cited:—

## I.

Per cent. by weight.

|                                    |    |
|------------------------------------|----|
| Ethyl alcohol                      | 52 |
| Ether                              | 46 |
| Mono-methylamin                    | 1  |
| Ethyl- or methyl-formate (or both) | 1  |

## II.

|                          | Per cent. by weight |
|--------------------------|---------------------|
| Ethyl alcohol            | 65                  |
| Ether                    | 34                  |
| 5 Mono- or di-methylamin | 0.5                 |
| Ethyl-formate            | 0.5                 |

## III.

|                       | Per cent. by weight |
|-----------------------|---------------------|
| 10 Ethyl alcohol      | 38 <sub>1</sub> –39 |
| Ether                 | 57                  |
| Di- or tri-methylamin | 3                   |
| Ethyl-formate         | 1–1 <sub>1</sub>    |

15 It will be seen that the relative proportions of the main components of the above fuels may be comparatively widely varied. When the proportion of amin is high (e. g. 2 or 3%) it is advantageous to use in conjunction with it the ethyl-formate only which is, it may be mentioned, the more effective deodorizer. It has been found that the invention permits, within certain limits, the use of a much larger proportion of 25 ether in such mixtures than would otherwise be possible. The use of formyl-esters in requisite proportions obviates any objectionable odor associated with the use of the fuels, and also inhibits the production 30 of deleterious acidic bodies produced by combustion.

The preferred order of mixing is first to dissolve the mono-methylamin in the alcohol, then to add the ethyl- or methyl-formate, and finally to add the ether.

The proportion of ether to alcohol and consequently the proportions of amin and ester employed therewith can conveniently be varied to suit the nature of the engine

(i. e., rotary aerial, small fixed engine, &c.) 40 and the nature of the carbureter.

What I claim as my invention and desire to secure by Letters Patent is:—

1. The herein described fuel composition which comprises a combustible liquid containing an aliphatic amin and a formyl ester. 45

2. The herein described fuel composition which comprises a combustible liquid containing a methylamin and a formyl ester. 50

3. The herein described fuel composition which consists of a mixture of alcohol and ether containing an aliphatic amin and a formyl ester.

4. The herein described fuel composition 55 which consists of a combustible liquid containing an aliphatic amin in the proportion of 0.5–3 per cent., and a formyl ester in the proportion of 0.5–2 per cent.

5. The herein described fuel composition 60 which consists of 38–70 per cent. of ethyl alcohol, 60–30 per cent. of ether, 0.5–3 per cent. of a methylamin and 0.5–2 per cent. of a formyl ester, by weight.

6. The herein described fuel composition 65 which consists of 52 per cent. ethyl alcohol, 46 per cent. ether, 1.0 per cent. of mono-methylamin and 1.0 per cent. ethyl formate, by weight.

7. The herein described fuel composition 70 which consists of ethyl alcohol in excess of 35 per cent., ether in excess of 30 per cent., mono-methylamin in excess of 0.5 per cent., ethyl formate in excess of 0.5 per cent., by weight.

In testimony whereof I affix my signature.

CHARLES LE PETIT.